

Sept. 18, 1934.

J. B. DECKER ET AL

1,974,015

PYROTECHNIC DEVICE

Filed March 22, 1932

*Fig. 1.*



*Fig. 2.*



Inventors

JOSEPH B. DECKER  
and HERBERT C. CLAUSER

By *Mason Tonwicke Lawrence*  
Attorneys

## UNITED STATES PATENT OFFICE

1,974,015

## PYROTECHNIC DEVICE

Joseph B. Decker and Herbert C. Clouser,  
Elkton, Md.

Application March 22, 1932, Serial No. 600,427

13 Claims. (Cl. 52—24)

This invention relates to fulminating pyrotechnic devices, and its object is the provision of an improved toy torpedo characterized by a loud detonation accompanied by a brilliant flash which may, if desired, be of different colors and interspersed with scintillating particles or stars.

A more specific object of the invention is the provision of a toy torpedo employing, as the fulminating composition, one or more of the group of elements hereinafter enumerated from the periodic group IVA and certain rare earth metals, in comminuted state, in mixture with an oxidizing agent.

Still another object of the invention is the inclusion in the fulminating composition of an ingredient imparting color to the flash.

A further object of the invention is the control of the fineness of comminution of the particles of the metal whereby, using a relatively coarse mesh, combustion of the particles is not instantaneous so that scintillating stars are thrown out into the field of the flash.

Another object of the invention is to increase the factor of safety in the manufacture and transportation of toy torpedoes.

Other objects of the invention will appear as the following description of a preferred and practical embodiment of the invention proceeds.

In the drawing which forms a part of the following specification, Figure 1 is a diametrical section through a torpedo embodying the principles of the invention; Figure 2 is a similar view showing the torpedo exploding.

In known processes for manufacturing toy torpedoes, an intimate mixture of potassium chlorate, antimony disulfid and sulphur in proper proportions is ordinarily employed as the fulminating agent, the same being mixed with abrasive granules such as pebbles, and enclosed in a shell or other gas confining container.

While such torpedoes are satisfactory with respect to the intensity of the detonation, they are not spectacular as to flash, nor are they amenable to coloration of the flash since the proportions in which the fulminating ingredients are sensitive to impact are rather critical, and the addition of a color ingredient to the mixture in any practical proportions, adulterates it sufficiently to impair or destroy its sensitivity to fulmination.

The ordinary potassium chlorate, antimony disulfid, sulphur composition must be thoroughly mixed to obtain the essential degree of

sensitivity but then the sensitivity is such that accidental explosions occasionally occur both in manufacture, and transportation notwithstanding the special packaging that is resorted to for the prevention of such calamities. 60

It was in the quest of a safer toy torpedo that the present invention was evolved, in which not only has a safer torpedo been produced, but one capable of a variety of spectacular effects which were not possible with the ordinary torpedo. 65

It has been found that certain members of the group of rare earth metals as well as certain elements of the periodic group IVA, of which zirconium, titanium, thorium, yttrium, selenium 70 are examples, or alloys of these metals, are particularly adapted for use as the reducing factor of a fulminating composition, in mixture with an oxidizing agent, of which substances, there is a wide range of availables, such for example 75 as potassium nitrate, barium nitrate, oxalates, trinitro compounds, chlorates, and perchlorates.

From this group may be selected an oxidant particularly adapted to cooperate with the metal or alloy of the same which may have 80 been adopted as the reducing element.

For example, one may select comminuted zirconium in the metallic state. This when mixed with barium nitrate in the ratio of two to three parts by weight, gives a fulminating composition which is notably stable in the process of mixing and also safe in transportation, particularly when the pebbles are agglomerated into a unitary mass which is disruptable only at a definite impact value, as covered in the application of Joseph B. Decker, Serial No. 591,213, filed February 5, 1932. 90

It is characteristic of the ingredients of this fulminating composition, that the zirconium or other of the aforementioned metals or alloys of the same enhances the sensitivity of the oxidant so that the latter may in itself be inert to impact, but be endowed with any desired value of sensitivity, by controlling the proportions of the rare earth metal or alloy. 100

Referring in detail to the drawing, the numeral 1 represents the torpedo, having a shell 2 forming a gas confining chamber in which is packed a mixture 4 of one of the detonating substances disclosed in the specification such 105 for example as zirconium, the same being interspersed with a mass of pebbles 3 producing the friction when shocked which detonates the torpedo.

In manufacturing the improved torpedo, the 110

zirconium and barium nitrate in proportions of substantially two parts to three parts by weight are mixed, and in view of the controlled sensitivity, they may be mixed in large quantity with impunity. The torpedo is made in the usual manner by mixing an appropriate charge of the fulminating composition with pebbles and loading the same into a gas confining container, or the mass of gravel may be first agglomerated in the manner previously suggested, and the interstices between the pebbles filled with the fulminating mixture.

It has been found that the addition of color producing ingredients to the mixture of the said metals or alloys and appropriate oxidants, in quantity sufficient to give satisfactory color effect to the flash, does not affect the fulminating sensitivity of the mixture as it does the fulminated composition ordinarily heretofore used, so that the new fulminating mixture lends itself readily to the production of spectacular colored flashes as an accompaniment to the detonation.

Since barium nitrate gives a green flash, it is not necessary to add another ingredient to produce this color, the barium nitrate functioning both as the oxidizing element and the color producing ingredient in mixture with the zirconium. The zirconium or equivalent metal or alloy being the reducing agent or fuel, gives a brilliance to the flash hitherto unobtainable in fulminating or combustible light producing compositions in which the rare earth metal or alloy may have played any other role.

In producing flashes of other colors than green, it is preferred to select an oxidant which produces an inherently white or uncolored flame so that the color of the added ingredient will remain pure and uncontaminated with any color native to the basic flash. The perchlorates are particularly adapted for oxidizing agents of the said metals and alloys when color producing ingredients are to be added, both by reason of the whiteness of the basic flame, and because the chlorine ions freed in the reaction vivify the flash, increasing its brilliancy. Moreover, a greater volume of gas is released than with other oxidants, thereby extending the field of the flash.

The following are examples of fulminating mixtures producing flashes having particular color effects:

- 50 Red:  
Zirconium  
Ammonium perchlorate  
Small quantity of strontium carbonate, lithium carbonate or calcium nitrate
- 55 Blue:  
Zirconium  
Ammonium perchlorate  
Copper sulfid
- 60 Yellow:  
Zirconium  
Ammonium perchlorate  
Sodium oxalate
- 65 Purple:  
Zirconium  
Potassium permanganate

Scintillating particles or stars in the flash are obtained by controlling the size of the comminution of the particles of the metal which may have been selected as the reducing and detonative agent. By making these sufficiently coarse, their combustion is not instantaneous but continues as they are thrown out into the field of flash from the focus of the explosion. Each

metal and metallic alloy appears to have a characteristic manner of combustion, and therefore, to give a definite characteristic visual effect in the spark. For instance, the zirconium star appears to be an incandescent area of amoeba-shaped contour as indicated at 5 in Figure 2. A modified form results from the combustion of an iron-zirconium alloy, the star points being more blunt and less deeply cut into the area of the star as indicated at 6 in Figure 2.

It is obvious from the above that we have produced a new and improved toy torpedo in which spectacular effects both as to intensity of flash and color of flash as well as the presence of scintillating stars are made to accompany the detonation, through the use of rare earth metals and alloys of the same as reducing agents, in mixture with oxidizing compounds, and that the factor of safety in the manufacture and transportation of torpedoes has been increased.

It is to be understood that while we have specified the fulminating composition as being formed with ingredients in different proportions, it is to be understood that these proportions may be varied substantially without departing from the spirit of the invention and that the examples included in the foregoing specification are to be regarded as illustrative and not as limitative in their bearing upon the scope of the invention which is to be determined by the claims appended hereto.

What we claim is:

1. Pyrotechnic device capable of detonating upon concussion, comprising means forming a gas confining chamber containing a mixture of an element selected from the following group: zirconium, titanium, thorium, yttrium, selenium, with an oxidizing agent.
2. Pyrotechnic device capable of detonating upon concussion comprising means forming a gas confining chamber containing abrasive material and a mixture of an element selected from the following group: zirconium, titanium, thorium, yttrium, selenium, with an oxidizing agent.
3. Pyrotechnic device capable of detonating upon concussion comprising means forming a gas confining chamber containing a mixture of an oxidizing agent, with a sensitivity accelerating proportion of an element selected from the following group: zirconium, titanium, thorium, yttrium, selenium.

4. Pyrotechnic device capable of detonating upon concussion comprising means forming a gas confining chamber, containing abrasive material and a mixture of oxidizing agent with an element selected from the following group: zirconium, titanium, thorium, yttrium, selenium in the ratio of substantially three to two.

5. Pyrotechnic device capable of detonating upon concussion comprising means forming a gas confining chamber, containing a mixture of an element selected from the following group: zirconium, titanium, thorium, yttrium, selenium, with an oxidizing agent, and a color imparting ingredient in such proportion as to give a decided color to the flash eventuating from the detonation of said mixture.

6. Pyrotechnic device capable of detonating upon concussion comprising means forming a gas confining chamber containing a mixture of an element selected from the following group: zirconium, titanium, thorium, yttrium, selenium, with an oxidizing agent, the said element being comminuted with such degree of coarseness as

to produce stars in the flash eventuating from the detonation of said mixture.

7. Pyrotechnic device capable of detonating upon concussion comprising means forming a gas confining chamber, an abrasive material in said chamber and a mixture of comminuted zirconium in metallic state with an oxidizing agent.

8. Pyrotechnic device as claimed in claim 7, the ratio of the zirconium to the oxidizing agent being substantially as three to two.

9. Pyrotechnic device as claimed in claim 7, the ratio of the zirconium to the oxidizing agent being substantially as three to two, and the zirconium being comminuted to such degree of coarseness as to produce stars in the flash eventuating from the detonation of the mixture.

10. Pyrotechnic device capable of detonating upon concussion comprising means forming a gas confining chamber, containing a mixture of zirconium, a perchlorate, and a color imparting ingredient, the latter being in such proportion to give a decided color to the flash eventuating from the detonation of said mixture, the perchlorate functioning as an oxidizing agent.

11. Pyrotechnic device with fulminating characteristic comprising means forming a gas confining chamber, containing a mixture of zirconium, a perchlorate, and a color producing ingredient, the perchlorate functioning as an oxidizing agent, and the zirconium being comminuted to a degree of coarseness producing stars in the field of the flash eventuating from the detonation of said mixture.

12. Pyrotechnic device capable of detonating upon concussion comprising means forming a gas confining chamber, containing a mixture of an element capable by itself of detonating upon concussion, and an oxidizing agent.

13. Pyrotechnic device capable of detonating upon concussion comprising means forming a gas confining chamber, containing a mixture of zirconium, an oxidizing agent, and a color imparting ingredient, the latter being in such proportion as to give a decided color to the flash eventuating from the detonation of said mixture.

JOSEPH B. DECKER.  
HERBERT C. CLAUSER.

80

85

90

95

100

105

110

115

120

125

130

135

140

145

150